

Patented Oct. 25, 1927.

## UNITED STATES PATENT OFFICE.

CHARLES A. HUTTINGER, OF LAKewood, OHIO, ASSIGNOR, BY MESNE ASSIGNMENTS,  
TO THE ACME RAYON CORPORATION, OF CLEVELAND, OHIO, A CORPORATION OF  
OHIO.

## PROCESS OF PRODUCING THREADS FROM VISCOSE.

No Drawing.

Application filed August 14, 1922. Serial No. 581,833.

My invention relates to processes of producing lustrous threads, etc., from viscose. This invention contemplates the production of a very soft and open thread. The invention relates particularly to the composition of the bath in which the viscose is regenerated into cellulose hydrate.

The following description sets forth in detail certain steps illustrating the method 10 of carrying out my invention, such disclosed steps constituting, however, but one of the various ways in which the principle of the invention may be utilized.

In carrying out my improved process, 15 I utilize a precipitating bath in the presence of a certain proportion of sugar. Also, I may incorporate the sugar with the precipitating bath. The proportion by weight of sugar may be from five to twenty per cent 20 but I have found that from seven to ten per cent gives the best results.

The precipitating bath, in addition to the sugar, consists of an aqueous solution of a semi-neutral sulfate salt and preferably of an aqueous solution of sodium bisulfate because the latter is a by-product which can be bought comparatively cheaply. The relative proportions which I use are substantially ten (10) parts by weight water, six 25 (6) parts bisulfate, and one and one-half (1½) parts sugar. I preferably utilize common granulated sugar, other factors, such as price, availability, etc., being equal. The exact proportions of a very satisfactory 30 bath will consist in one kilogram water, 63½ grams sodium bisulfate and 164 grams common granulated sugar.

The thread obtained by spinning the multiple filaments of cellulose hydrate precipitated by a bath of the character disclosed is a product which has the necessary qualities as regards luster, strength and elasticity, and is also unusually soft and open. My

theory is that the extraordinary softness and openness is occasioned by the following 45 physical action of the sugar while the filaments are setting in the precipitating bath. The sugar exteriorly coats the several strands of the viscose while the same is setting, possibly somewhat analogous to the 50 coating of flour on a rolling board whereby the dough is prevented from sticking, so that the multiplicity of strands,—from ten to sixty or more, according to the thread produced,—do not stick or closely adhere 55 when being twisted. This coating of sugar is washed off in the usual water washing after the skein is formed and the resultant product is the very soft and open thread which has been mentioned. By the time 60 the coating of sugar has been washed off, the filaments have so hardened that they will not closely adhere.

What I claim is:

1. In the process of producing threads 65 from viscose, the steps which consist, in introducing the latter in multiple streams into a precipitating bath composed of substantially ten (10) parts by weight water, six (6) parts sodium bisulfate, and one and one-half (1½) parts sugar; and then spinning the resultant filaments, whereby a soft and open thread is obtained.

2. In the process of producing threads 75 from viscose, the steps which consist, in introducing the latter in multiple streams into a precipitating bath composed of substantially one thousand (1000) parts by weight water; six hundred and thirty-one (631) parts sodium bisulfate, and one hundred and sixty-four (164) parts granulated sugar; and then spinning the resultant filaments, whereby a soft and open thread is obtained.

Signed by me, this 27th day of July, 1922.  
CHARLES A. HUTTINGER.